

March 18, 1924:

J. R. STACK

1,487,125

PROCESS OF RECOVERING TIN

Original Filed Jan. 4, 1922



INVENTOR

James Robert Stack  
BY  
Albert M. Austin

ATTORNEY

## UNITED STATES PATENT OFFICE.

JAMES ROBERT STACK, OF PERTH AMBOY, NEW JERSEY.

## PROCESS OF RECOVERING TIN.

Application filed January 4, 1922, Serial No. 526,871. Renewed January 14, 1924.

To all whom it may concern:

Be it known that I, JAMES ROBERT STACK, a citizen of the United States, and resident of Perth Amboy, in the county of Middlesex and State of New Jersey, have invented certain new and useful Improvements in Processes of Recovering Tin, of which the following is a specification.

This invention relates generally to a process for the treatment of complex bullion and alloys containing tin, bismuth and similar metals to recover the values contained therein.

My method, considered broadly, comprises a method of separating and recovering certain metals and particularly bismuth and tin from complex alloys containing lead, copper, antimony, arsenic and the precious metals, by subjecting the impure bullion or alloy to electrolysis under conditions that will cause the bismuth and tin to remain in solution and the other metals to be precipitated with the slimes, and then separating the bismuth and tin.

The process also comprises an improved method of separating the tin and bismuth remaining in solution after their separation from other metals, such as lead, copper, antimony and the like, by precipitating the bismuth either as a commercial product or as a compound susceptible of treatment by standard methods to produce a commercial product, and then recovering the tin in a commercial condition.

The invention further consists in treating impure bullion and alloys containing bismuth and tin by a practically continuous process that first separates the bismuth and the tin by precipitating all or substantially all of the lead, copper, antimony, arsenic and the precious metals by electrolysis and causes such metals to be deposited as slimes in the form of compounds or alloys easily refined to produce commercial products; then by chemical substitution precipitates the bismuth and any traces remaining of the other metals to produce a solution containing tin in the form of a salt, and finally recovers the tin in commercial form from the solution.

Although the process may be utilized in the treatment of impure alloys and bullions containing various complex mixtures of

metals, it will be described with special reference to the treatment of slimes recovered in the electrolysis of impure tin bullion produced by reduction of Bolivian or Colombian ores, which contain a large number of other metals in greater or less amounts, in addition to the tin and bismuth content. Relatively large quantities of anode slimes are produced in the primary treatment of such impure bullion, which contain appreciable quantities of tin occluded with the other metals. In practice approximately seven to ten per cent of anode slimes are produced for each ton of bullion treated, and these slimes occlude approximately two per cent of the total amount of tin contained in the ore. A considerable portion of the lead present in the slimes, for example, as high as 50%, may be present as lead sulphate, and part of the tin is present as finely divided metallic tin. The remaining portion of the tin and of the lead, together with the other metals found in the ore, form a complex alloy.

In practice the slimes are first smelted to complete reduction in a suitable reverberatory or blast furnace. About 1400 to 1500 pounds of metallic alloy will be made from one ton of slimes. This alloy is cast into anode plates of suitable dimensions and weight that will have approximately the following composition:

|    |      |               |
|----|------|---------------|
| Au | .165 | ozs. per ton. |
| Ag | 178. | " " "         |
| Pb | 16%  |               |
| Cu | 6%   |               |
| As | 5%   |               |
| Sb | 3%   |               |
| Sn | 34%  |               |
| Bi | 35%  |               |

Reference is made to the drawing, which shows a flow sheet illustrative of the steps of the process hereinafter described.

Referring to the drawing, the plates 2 as anode are then subjected to electrolysis in a vat 4 of any suitable or well known construction. The cathode 6 may be a sheet of lead, copper, iron or of tin, and it is separated from the anode by a semi-permeable partition or membrane 8 of any preferred construction,—for example, by being inserted in an unglazed clay cell that will prevent

mechanical mixing or diffusion of the electrolyte while permitting passage of the current by migration or ionic diffusion. The anolyte 10 may be hydrochloric acid solution containing approximately 18% acid. Preferably the cathode electrolyte 12 is also a hydrochloric acid solution. Various other acids, such as sulphuric acid and compounds, may be substituted if desired as anolyte or cathode, provided only the electrolyte is adapted to take both tin and bismuth into solution upon the passage of the electrolytic current.

During electrolysis the temperature of the electrolyte is maintained approximately at 100° F., while stratification is prevented by circulation or other suitable means. A direct current of about 550 amperes is applied, corresponding to a current density of approximately 20 amperes per square foot of anode surface with a voltage of approximately 2%. Both the amperage and the voltage may vary somewhat depending on the constituents of the anode, the composition of the electrolyte and the temperature, and good results have been obtained with a density of from 20 to 30 amperes and a voltage of from one and one-half to two and one-half volts.

30 The metals of the anode gradually dissolve, not however according to the potential series, but as a complex alloy of bismuth, tin, antimony, copper, arsenic and lead. The lead will be precipitated in the cool, moderately dilute hydrochloric acid solution as  $PbCl_2$ , which is insoluble and falls to the bottom of the tank with the slimes. The arsenic will also be precipitated in the metallic state by tin chloride, the reaction being approximately as follows:



45 All of the gold and silver and substantially all of the lead, copper, arsenic and antimony are thus contained in the slimes which settle to the bottom of the tank and may be removed and treated in any suitable way for the recovery of these metals. Preferably the slimes are filter pressed and then subjected to any one of the numerous methods now in common use, such, for example, as the methods employed in refining or softening and liquating lead, which will result in the complete separation of the metals with recovery of the total values contained.

55 The reactions are not to be understood as being absolutely quantitative, however, because negligible percentages of lead and arsenic may remain in the solution and be removed later, as hereinafter described. When the solution has become saturated with metallic salts, it is removed for subsequent treatment to recover the dissolved metals. In case the anodes have not been 65 totally dissolved, fresh acid solution may

be added and the treatment continued until the anodes are reduced to scrap.

The saturated solution after removal from the electrolyzing vat 4 is conducted to a precipitation tank 14 of any desired construction, is heated to a temperature of about 110° F., and preferably is vigorously agitated by air introduced under slight pressure. A quantity of metallic tin or other metal or metals above bismuth in the E. M. F. series is then added to the solution, which causes relatively rapid precipitation of the bismuth and any remaining copper, arsenic, and antimony in a finely divided form known as bismuth cement. The solution in which the metallic equivalent of tin, in place of the other metals, has been dissolved is then allowed to cool and settle and the supernatant liquid decanted. The bismuth cement that settles to the bottom of the tank can be refined by any well known process, and without further treatment, can be disposed of as a standard product of commerce.

60 The liquid decanted will contain approximately from twelve to fifteen per cent of tin in the form of tin chloride, and will be entirely free from other metals except slight traces which may be removed by the addition of fresh acid and a longer period of treatment, or which may be disregarded, as they do not affect the commercial value of the final product. The tin chloride can be reduced to a commercial product by various methods or it may be evaporated and sold as 100 bichloride of tin solution, or the tin chloride may be crystallized and the crystals marketed. If it is desired to produce metallic tin, this may be accomplished in various 105 ways, for example, by evaporating the chloride solution to a small bulk and mixing the same with calcium oxide to a thick paste, which is allowed to set, and is then smelted for the recovery of metallic tin.

110 By my improved process the tin is recovered in a state of unusual purity without being subjected to metallurgical processes to refine the metal and remove impurities therefrom. The metals arrange themselves in each of the steps of the process in groups which are readily reduced and separated without the formation of further complex or refractory alloys. The lead, copper and arsenic are almost completely removed in the first step of the operation with the slimes precipitated at the bottom of the electrolytic vat. The antimony and the other metals that may remain in small amount are separated and removed with the bismuth as a bismuth cement, which is also readily treated to separate the constituent metals according to well known standard practice for the refining of such material. Consequently the process possesses marked advantages not only because of the high purity 115 120 125 130

of the final products obtained but also because the intermediate and secondary products of the several steps toward the desired result are of a character and of a composition which will permit them readily to be assimilated in the practice of established commercial metallurgical plants.

Although I have shown and described and have pointed out in the annexed claims, certain novel features of my invention, it will be understood that various omissions, substitutions and changes in the several steps of my process and in its operation may be made by those skilled in the art without departing from the spirit of the invention.

What I claim is:

1. The process of refining impure tin bullion to recover the contained metals, which consists in subjecting the bullion as anode to an electrolytic current of appropriate voltage and amperage in an electrolyte capable of holding tin and bismuth in solution and depositing substantially all of the other contained metals as slimes or precipitates, and then separating the tin from the bismuth and other metals by precipitating the bismuth and retaining the tin in solution.

2. The process of refining impure tin bullion to recover the contained metals, which consists in passing a current of appropriate voltage and amperage from the bullion as anode to a cathode separated from the anode by a semi-permeable membrane through an electrolyte capable of combining with tin and bismuth to form soluble salts and which will deposit a substantial portion of each of the remaining metals as slimes, then precipitating the bismuth and other metals by adding an excess of tin to the solution and treating said solution and the slimes separately to recover the metal values thereof.

3. The process of refining impure tin bullion to recover the contained metals, which consists in passing an electrolytic current from the bullion as anode to a cathode separated from the anode by a diaphragm permitting ionic diffusion through an electrolyte capable of holding tin and bismuth in solution, which will form a non-soluble salt of lead and react with the compounds of arsenic to deposit metallic arsenic as slimes, then adding an excess of tin to the electrolyte to precipitate bismuth and other metals contained therein, and recovering the values contained in said slimes and solution.

4. In the electrolytic refining of complex alloys containing tin, bismuth and lead, the method of separating tin and bismuth which consists in passing a current of appropriate voltage and amperage from the alloy as anode to a cathode separated from the anode by a semi-permeable membrane through an electrolyte which will take the tin and bismuth into solution and precipitate the lead as a non-soluble salt, and then separating

the tin by adding a precipitating agent to the solution to form a non-soluble bismuth cement.

5. In the electrolytic refining of complex alloys the method of forming a bismuth cement from the electrolyte containing tin, bismuth and other metals in solution, which consists in passing an electrolytic current of approximately 20 to 30 amperes and one to two volts from the alloy as an anode to a cathode separated from the anode by a porous diaphragm through an electrolyte which will combine with lead and arsenic and retain the tin and bismuth in solution, and then adding an excess of tin to precipitate the bismuth and metals other than tin as a bismuth cement.

6. In the electrolytic refining of complex alloys to recover tin, the method which consists in passing an electrolytic current having a voltage of approximately one-half to two volts and a current density of from 20 to 30 amperes from the alloy as anode to the cathode separated by a semi-permeable diaphragm through an electrolyte adapted to hold the tin in solution, removing the solution from the slimes, heating the same to a temperature of approximately 110° F., adding an excess of metallic tin to the solution to precipitate the other metals contained therein, and then recovering the tin.

7. In the electrolytic refining of impure bullion and complex alloys to recover tin, the method which consists in passing an electrolytic current of approximately 20 to 30 amperes and one to two volts from the alloy as anode to a cathode electrolytically insulated from the anode through an electrolyte heated approximately to 100° F., which takes the tin and bismuth into solution on the passing of the current, removing the solution and heating the same approximately to 110° F., precipitating the bismuth, antimony, arsenic and copper as a bismuth cement and then recovering the tin.

8. In the electrolytic refining of complex alloys the method which consists in separating the gold, silver, lead and arsenic and a portion of the copper and antimony from tin and bismuth by passing a current of appropriate amperage and voltage from the alloy as anode to a cathode separated from the anode by a semi-permeable membrane through an electrolyte containing hydrochloric acid heated to a temperature of 100° F., until the tin, bismuth and portions of the other metals are dissolved, removing the solution with the dissolved metals, heating the same to a temperature of approximately 110° F., precipitating the bismuth, arsenic, antimony and copper as a bismuth cement and then recovering the tin.

9. In the electrolytic treatment of complex alloys containing tin and bismuth to recover and separate the metals therein, the

method which consists in subjecting the alloy as anode to an electrolytic current having a current density of approximately 20 to 30 amperes and from one to two volts through an electrolyte adapted to take tin and bismuth into solution on the passage of the current and to precipitate lead and arsenic, interposing a porous diaphragm between the cathode and the anode during electrolysis, then removing the solution and heating the same to a temperature of approximately 110° F. and agitating the same with air, adding a metal having a higher potential than bismuth to precipitate any antimony, arsenic, copper and bismuth as a bismuth cement, and then recovering the tin from the solution.

10. In the electrolytic treatment of anode slimes to separate the metals contained therein, the process which comprises the smelting of the slimes to a metallic state and casting the same into anode plates, passing a current from said plate as an anode to a cathode separated from the anode by a semi-permeable diaphragm through an electrolyte capable of combining with lead to form an insoluble salt and to hold the tin and bismuth

in solution, precipitating the bismuth as a cement by adding an excess of metallic tin to the solution and then recovering the tin. 30

11. In the electrolytic treatment of anode slimes containing tin, bismuth, lead, arsenic and the precious metals, to recover the metals contained therein, the process which comprises the smelting of the slimes to a metallic state and casting the same into anode plates, passing a current of appropriate voltage and amperage from said plates as anodes to cathodes separated from the anode by a porous diaphragm through an anolyte containing approximately 18% of hydrochloric acid to take the tin and bismuth in solution and deposit metallic gold, silver, arsenic and insoluble salts of lead as slimes, separating the slimes from the solution, adding a metal having a higher potential than bismuth to precipitate the metals having a lower potential contained in the solution, and then treating said solution to recover the tin. 45

Signed at Perth Amboy, in the county of Middlesex and State of New Jersey, this 30th day of December, A. D. 1921.

JAMES ROBERT STACK.